

# United States Patent [19]

Asano et al.

[11] 3,912,601

[45] Oct. 14, 1975

[54] **SURFACE TREATMENT OF TIN-PLATED STEEL SHEETS**

[75] Inventors: **Hidejiro Asano; Yoshitaka Hiromae**,  
both of Kitakyushu, Japan

[73] Assignee: **Nippon Steel Corporation**, Japan

[22] Filed: **July 18, 1974**

[21] Appl. No.: **489,489**

[30] **Foreign Application Priority Data**

Aug. 1, 1973 Japan ..... 48-86622

[52] **U.S. Cl.** ..... 204/56 R; 204/35 R; 204/40

[51] **Int. Cl.<sup>2</sup>** ..... C25D 11/36

[58] **Field of Search** ..... 204/35 R, 56 R, 54, 40

[56] **References Cited**

UNITED STATES PATENTS

3,616,307 10/1971 Snyder ..... 204/56 R

FOREIGN PATENTS OR APPLICATIONS

698,632 11/1964 Canada ..... 204/35 R

*Primary Examiner*—R. L. Andrews  
*Attorney, Agent, or Firm*—Toren, McGeady and  
Stanger

[57]

**ABSTRACT**

A surface treatment of a tin-plated steel sheet which comprises electrolyzing the tin-plated steel sheet as cathode with a quantity of electricity between 1 and 50 c/dm<sup>2</sup> in an aqueous solution containing 1 to 50 g/l of at least one of aluminum dihydrogenphosphate, aluminum monohydrogenphosphate and their mixture.

**2 Claims, No Drawings**

## SURFACE TREATMENT OF TIN-PLATED STEEL SHEETS

The present invention relates to surface treatment of tin-plated steel sheets, and more particularly relates to the surface treatment of tin-plated steel sheets for the purpose of prevention of damage to the sheet otherwise caused during a can-making process or during transportation.

Conventionally, electro-tin-plated steel sheets are subject to a passivation treatment after electro-tin-plating in order to prevent oxidation of the surface of the tin-plated steel sheet.

As for the passivation treatment, an electrolytic treatment in a sodium bichromate bath has been widely used. This electrolytic treatment, although very useful for preventing abnormal increase of the tin oxide, has a defect in that a small amount of chromium oxide in the surface adheres and accumulates on the piler and tools in the can-making line and causes damages to the surface of the tin-plated steel sheet.

In order to eliminate the above defect, lubricating oil is applied on the surface of the tin-plated steel sheet, but complete prevention of the surface damage can not be attained because the amount of the oil coating is limited for other reasons.

The surface damage deteriorates not only the outer appearance of a can but also its corrosion resistance. Therefore, there has been a strong demand for development of a complete method for preventing the surface damage which satisfies both the productivity and economy requirements.

The present inventors have conducted various studies and experiments on surface treatments which satisfy the oxidation (passivation) of tin and are effective to prevent the surface damage, and have discovered that the formation of a phosphate film is most effective for this purpose. Then the present inventors have con-

The reason for limiting the concentration of aluminum dihydrogenphosphate  $Al_2(H_2PO_4)_3$ , aluminum monohydrogenphosphate  $Al_2(HPO_4)_3$  or their mixture to the range from 1 to 50 g/l is that if the concentration is less than 1 g/l, an effective film for preventing the surface damage is not formed and if the concentration is more than 50 g/l, there is a tendency for deterioration of the surface brightness other than the surface damage problem.

Meanwhile, the pH value of the aqueous solution is maintained to 3 or less since if the pH value exceeds 3, the surface brightness is deteriorated.

As for the bath temperature, better results can be obtained when it is between 20 and 80°C.

When the tin-plated steel sheet is electrolyzed as a cathode under the above conditions, this treatment is performed with a quantity of electricity between 1  $c/dm^2$  and 50  $c/dm^2$ . When the quantity of electricity is less than 1  $c/dm^2$ , oxidation resistance of the tin-plated steel sheet is unsatisfactory and on the other hand when it is larger than 50  $c/dm^2$ , the outer appearance of the tin-plated steel sheet deteriorates and solderability of the sheet is poor.

The tin-plated steel sheet, when treated under the above conditions, possesses very excellent properties.

The present invention will be more clearly understood from the following examples.

### EXAMPLE 1

A low carbon steel sheet of 0.23 mm thickness produced from an ordinary method was degreased in a caustic soda solution and then acid-pickled in a sulfuric acid solution. The surface-cleaned steel sheet was subjected to electro-tin-plating in a stannous phenolsulfonate electrolyte to give a tin coating of 12  $g/m^2$ , the thus tin-plated steel sheet heated to 270°C to melt the tin to obtain mirror brightness, and then treated under the following conditions.

|                          |                               |                     |
|--------------------------|-------------------------------|---------------------|
| Treating bath:           | aluminum bishydrogenphosphate | 20 g/l              |
| Temperature:             | pH                            | 2                   |
| Electrolysis conditions: | 50°C                          |                     |
|                          | Current density               | 4 A/dm <sup>2</sup> |
|                          | Time                          | 2 seconds           |

ducted further studies on a method for forming the phosphate film and have found that the film is formed when a tin-plated steel sheet is electrolyzed as a cathode in an aqueous solution containing 1 to 50 g/l of aluminum dihydrogenphosphate or aluminum monohydrogenphosphate (or their mixture) which has a pH value not larger than 3.

The tin-plated steel sheet was electrolyzed as a cathode with a direct current.

### EXAMPLE 2:

A tin-plated steel sheet prepared by the method of Example 1 was treated as a cathode under the following conditions.

|                           |                                |                     |
|---------------------------|--------------------------------|---------------------|
| Treating bath :           | Aluminum monohydrogenphosphate | 30 g/l              |
|                           | Phosphoric acid                | 10 g/l              |
|                           | pH                             | 1.7                 |
| Temperature :             | 70°C                           |                     |
| Electrolysis conditions : | Current density                | 8 A/dm <sup>2</sup> |
|                           | Time                           | 2 seconds           |

## EXAMPLE 3:

A tin-plated steel sheet prepared by the method of Example 1 was treated as a cathode under the following conditions.

Treating bath: Aluminum dihydrogenphosphate 10 g/l  
pH 2.5  
Temperature: 35°C  
Electrolysis conditions: Current density 15 A/dm<sup>2</sup>  
Time 2 seconds

## EXAMPLE 4:

A tin-plated steel sheet prepared by the method of Example 1 was treated as a cathode under the following conditions.

Treating bath: Aluminum monohydrogenphosphate 10 g/l  
Aluminum dihydrogenphosphate 10 g/l  
pH 2  
Temperature: 70°C  
Electrolysis conditions: Current density 5 A/dm<sup>2</sup>  
Time 2 seconds

5

## EXAMPLE 6:

A tin-plated steel sheet prepared by the same method as in Example 1 was treated as a cathode under the following conditions.

Treating bath: Sodium bichromate 25 g/l  
pH 5  
Temperature: 50°C  
Electrolysis conditions: Current density 5 A/dm<sup>2</sup>  
Time 2 seconds

Properties of the tin-plated steel sheets treated by the above examples are shown in Table 1. It is clearly understood from the table that the tin-plated steel sheets treated by the method according to the present invention show better oxidation resistance and remarkably better surface properties.

Table 1

|                        | Example No. | Surface-damage Resistance | Oxidation Resistance | Solderability | Lacquerability | Yellow-coloration Resistance |
|------------------------|-------------|---------------------------|----------------------|---------------|----------------|------------------------------|
| Present Invention      | 1           | ◎                         | ◎                    | ◎             | ◎              | ◎                            |
|                        | 2           | ◎                         | ◎                    | ◎             | ◎              | ◎                            |
|                        | 3           | ◎                         | ◎                    | ◎             | ◎              | ○                            |
|                        | 4           | ◎                         | ◎                    | ◎             | ◎              | ◎                            |
|                        | 5           | ◎                         | ◎                    | ◎             | ◎              | ◎                            |
| Conventional Treatment | 6           | X                         | ○                    | ○             | ○              | ○                            |

◎ : Excellent

○ : Good

X : Not good

## EXAMPLE 5:

A tin-plated steel sheet prepared by the same method as in Example 1 was treated as a cathode in a 0.5% sodium carbonate solution for 2 seconds with a current density of 5 A/dm<sup>2</sup>, and then treated as a cathode under the following conditions.

Treating bath: Aluminum monohydrogenphosphate 20 g/l  
Phosphoric acid 10 g/l  
pH 2  
Temperature: 70°C  
Electrolysis conditions: Current density 5 A/dm<sup>2</sup>  
Time 2 seconds

45 What is claimed is:

1. A surface treatment of a tin-plated steel sheet which comprises electrolyzing the tin-plated steel sheet as a cathode with a quantity of electricity between 1 and 50 c/dm<sup>2</sup> in an aqueous solution containing 1 to 50 g/l of at least one of aluminum dihydrogenphosphate, aluminum monohydrogenphosphate and their mixtures, having a pH of 3 or less.

2. A surface treatment according to claim 1 in which the aqueous solution further contains phosphoric acid.

55

\* \* \* \* \*